

2,741,827

**PROCESS FOR THE MANUFACTURE OF PISTON RINGS BY POWDER METALLURGY AND ARTICLES OBTAINED THEREBY**

Max Koehler, Herbede (Ruhr), Germany, assignor to August H. Schilling, Atherton, Calif.

No Drawing. Application December 22, 1950,  
Serial No. 202,395

9 Claims. (Cl. 29—182)

The present invention relates to the manufacture of piston rings for high speed internal combustion engines based upon the pressing and sintering of mixtures of metallic powders, the main ingredient of which is powdered iron, and containing minor proportions of powdered lead and graphite.

In the known production of objects, for example, piston rings, by the powder metallurgical process, the metal powder is usually subjected to a pressing with a subsequent sintering, that is, a heat treatment wherein the temperature lies considerably under the melting point of the powdered metal mixture. In this type of manufacture, it is well known that the strength of the thus produced sintered body can be increased by the addition of small percentages of manganese, chromium or silicon to the soft iron powder. It has also been attempted to increase the strength of the resultant material by cold-pressing the same subsequent to the sintering or by subjecting it to several sintering treatments. No noteworthy increase in the material strength has, however, been attained by these processes.

Experience has shown, however, that piston rings manufactured according to the above suggestions are not entirely satisfactory for use in high speed internal combustion engines, for the latter impose very high thermal and mechanical stresses upon the rings.

It is the general object of the present invention to provide an improved process for the manufacture of piston rings and other parts for use in engines operating at high speed and at high temperatures.

More specifically, it is an object of the invention to provide an improved process whereby a material suitable for the manufacture of piston rings for high speed internal combustion engines is obtained and in which the crystal structure can be controlled by suitable modifications of the process.

It is a further object of the invention to provide an improved process for the manufacture of piston ring material by powder metallurgy wherein a mixture containing from 1% to 10% of lead with or without other heavy metals and silicon components all in powdered condition in admixture with powdered iron and a small proportion of powdered graphite, is converted into an extremely strong and heat resistant body, having exceptional bearing qualities by sintering and pressing, and in such manner that the material is given a lamellar pearlitic or a granular pearlitic or sorbitic structure.

Other objects and advantages of the invention will appear more fully from the following more detailed description thereof.

According to the present invention, powdered iron is ticketed or preliminarily pressed to approximately the desired final shape after mixing with a small proportion of powdered graphite and with 1% to 10% of powdered lead which may be replaced in part with one or more other heavy metals (i. e., metals having an atomic weight above 0) with or without silicon, until the specific gravity of the mass is about 6.3 to 6.5. This mass is then sintered

at a temperature of about 1000° to 1200° C., depending upon the fusion point of the added metal or metals, for a period of about one to two hours. The mass is then subjected to pressure at temperatures and under pressures dependent upon the structure it is desired to create in the finished mass and upon the use to which it is to be put.

In all cases, however, the sintered mass is subjected both to high pressure and either simultaneously with the pressing or subsequently thereto is brought to a temperature in the range of about 850° to 1000° C., i. e. above the transition or transformation temperature, after which it is either rapidly quenched, where the material is to be subjected in use to temperatures up to about 300° C. under load, or it is allowed to cool slowly where it is to be subjected to maximum temperatures of about 200° C. under load.

When additions of other heavy metals such as tin, antimony, manganese, chromium, nickel and copper, and also of silicon, are used along with the lead, the ratio of the additions to the quantity of lead must be so regulated that the diffusion processes internal to the mixed crystalline series structure like

Fe—Pb—Si, and Fe—Pb—Sb—Sn

are prevented.

My improved process may be varied in several ways for controlling the properties of the final product. In one modification of my process, it is sought to obtain a granular pearlitic or sorbitic structure which is particularly desirable for piston rings subject to high thermal stress in high-load, high-speed internal combustion engines, for example, those in which the operating piston ring temperature reaches approximately 300° C. In a modified procedure, it is desired to attain a fine lamellar pearlitic structure which is particularly desirable for the piston rings of high speed internal combustion engines which are operated at a thermally lower stress, where the ring temperatures do not exceed approximately 200° C.

The lamellar pearlitic structure is attained when, in the production of the piston ring material, iron powder containing a small proportion of graphite is mixed with a heavy metal powder consisting entirely or preponderantly of lead, with or without silicon, in the limits of 1 to 10%, preferably about 5%, which mixture is first pressed to a specific gravity of approximately 6.3 to 6.5 and then sintered at 1000° to 1200° C. for one to two hours and subsequently subjected to a hot-pressing at from 900° to 1000° C. and about 85,000 to 100,000 lbs./in.<sup>2</sup> (6,000 to 7,000 kg./cm.<sup>2</sup>) with a final slow cooling, for example, in air or an inert gas.

A lamellar pearlitic structure can also be obtained when the briquette of the above composition (specific weight 6.3 to 6.5) is sintered for from one to two hours at 1000° to 1200° C. followed by a step-wise cold-pressing to a final pressure of about 140,000 lbs./in.<sup>2</sup> (10,000 kg./cm.<sup>2</sup>) to a specific weight of 7.6 to 7.7 and with a final heating to 850° to 900° C. for approximately one hour, followed by a slow cooling. This lamellar pearlitic structure is particularly desirable for piston rings for high speed internal combustion engines operating under thermal stresses of the order of approximately 200° C.

For piston rings for high speed internal combustion engines with thermally more highly stressed rings, for example, where the piston ring operating temperature is approximately 300° C., the following manufacturing procedure will give the desirable granular pearlitic or sorbitic structure to the piston ring material.

The above-mentioned mixture is first consolidated to a specific gravity of 6.3 to 6.5, then sintered for one to two hours at 1000° to 1200° C. and subsequently hot-pressed at a temperature 900° to 1000° C. and a pressure of about 85,000 to 100,000 lbs./in.<sup>2</sup> by which a specific gravity of 7.6 to 7.7 is attained. This is followed by a

heat treatment at 800° to 850° C. with rapid quenching, for example, in oil. In a modification of my process for attaining this type of material with a granular pearlitic structure, there are carried out the above briquetting and sintering for one to two hours at 1000° to 12000° C., and these steps are followed by a step-wise cold-pressing to about 140,000 lbs./in.<sup>2</sup>, by which a specific gravity of 7.6 to 7.7 is obtained. After a subsequent heat treatment at 850° to 900° C. for approximately one hour, a rapid quenching is carried out, for example, in oil.

This last described process can be altered in that cold-pressing occurs in stages up to pressures of about 210,000 lbs./in.<sup>2</sup> (15,000 kg./cm.<sup>2</sup>) and that after a rapid quenching from approximately 800° C. a further soaking occurs at a temperature from 500° to 650° C., in any temperatures lying under the transition point of approximately 720° C. In further explanation the following may be noted:

During the cold-pressing, the cementite as well as the free graphite still present, and the mixed crystals of the Fe-C-heavy metal group, which were formed by the sintering subsequent to the briquetting, are distributed. In consequence, a rapid conversion into martensite is obtained by the subsequent heating to 760° to 820° C. with the rapid quenching that follows. With the subsequent soaking at temperatures of approximately 650° C., a grain structure build-up results whose special characteristic is annealed sorbite. This gives to the material the characteristics which are valuable for piston rings; namely, a higher elastic limit, strength and a springiness as well as extremely good running and slipping characteristics as yet not attained by any other process. The length of time required by the soaking must be determined by the cross section of the material and the desired strength; the time increases with larger cross sections and for the reaching of higher strengths.

The following example will serve to illustrate the invention more specifically without, however, indicating the limits thereof.

#### Example I

The following materials were mixed together:

|                                     | Percent |
|-------------------------------------|---------|
| Powdered iron                       | 93      |
| Powdered graphite (ash content 15%) | 1.5     |
| Powdered lead with additives        | 4.5     |

which mixture had the following approximate grain size distribution:

|                         | Percent |
|-------------------------|---------|
| under 0.06 mm           | 20      |
| between 0.06 and 0.1 mm | 39      |
| between 0.1 and 0.2 mm  | 26      |
| over 0.2 mm             | 15      |

The initial pressing or briquetting of this material occurred at a pressure of about 70,000 lbs./in.<sup>2</sup> (4,900 kg./cm.<sup>2</sup>) followed by sintering at approximately 1100° C. for two hours in a neutral furnace atmosphere. This crude sintered mass had a porosity of approximately 23% and an ultimate strength of 14,000 to 17,000 lbs./in.<sup>2</sup> (10 to 12 kg./mm.<sup>2</sup>).

This material was subsequently pressed at a temperature of 1000° C. and a pressure of about 100,000 lbs./in.<sup>2</sup>, the temperature having been attained in a protective atmosphere, and the material then allowed to cool slowly. This material had a definite fine lamellar pearlitic structure and the characteristics tabulated below under the heading "Example I."

#### Example II

The same mixture as in Example I, after sintering, was cold-pressed in stages until a maximum pressure of about 140,000 lbs./in.<sup>2</sup> (9,800 kg./cm.<sup>2</sup>) was reached. This material was subsequently heated and held for one hour at a temperature of 850° C. (The effect attained by this

heating may be developed in a shorter time by the use of a higher temperature, which temperature, however, may not exceed the sintering temperature.) At the end of this annealing, the material was oil quenched and examination showed it had a definite grainy pearlitic structure, and the characteristics tabulated below under the heading "Example II."

|                                               | Example I                             | Example II                            |
|-----------------------------------------------|---------------------------------------|---------------------------------------|
| 10 Elastic limit, kg./mm. <sup>2</sup> -----  | 57.5 (82,000 lbs./in. <sup>2</sup> )  | 62.6 (89,000 lbs./in. <sup>2</sup> )  |
| Ultimate strength, kg./mm. <sup>2</sup> ----- | 76.5 (109,000 lbs./in. <sup>2</sup> ) | 74.5 (106,000 lbs./in. <sup>2</sup> ) |
| 15 Elongation-----                            | 1.5                                   | 2.                                    |
| Chemical Analysis:                            |                                       |                                       |
| C-----                                        | 0.48%                                 | 0.52%                                 |
| Si-----                                       | 0.17%                                 | 0.16%                                 |
| Mn-----                                       | 0.18%                                 | 0.19%                                 |
| P-----                                        | 0.029%                                | 0.003%                                |
| Pb-----                                       | 3.55%                                 | 3.45%                                 |
| Sn-----                                       | 0.41%                                 | 0.36%                                 |
| Cu-----                                       | 0.45%                                 | 0.52%                                 |
| Fe-----                                       | remainder (approx. 94.7%).            | remainder (approx. 94.7%).            |

While in the foregoing, I have referred specifically to iron as the ferrous component, it will be understood that 25 various suitable types of steel can be employed, in place of various forms of iron, suitable adjustment of the quantity of graphite being made where necessary.

The term "heavy metal" or "heavy metal powder" as 30 employed in the specification and claims is to be understood as having reference to a solid metal of an atomic weight above 50 and of the type commonly employed in the metallurgy of iron and steel, and in minor proportions with reference to the iron, in order to modify the properties of the essentially ferrous product. The lead, tin, 35 antimony, manganese, chromium, nickel, and copper referred to hereinabove are typical examples of additions in modified iron and steel products and ferrous alloys.

I claim:

1. In a process for the manufacture of piston rings by powder metallurgy and suitable for use in high speed internal combustion engines, the steps which include pressing a mixture comprising a preponderating proportion of iron powder, about 1 to 10% of lead powder, and a small proportion of graphite to approximately the desired shape, 45 sintering the mass, and subsequently hot-pressing the same.
2. Process according to claim 1 including the subsequent step of slowly cooling the mass from an elevated temperature to produce a lamellar pearlitic structure.
3. Process according to claim 1, including the subsequent step of quenching the mass from an elevated temperature to produce a granular structure of the type of pearlite and sorbite.
4. In a process for the manufacture of piston rings by powder metallurgy and suitable for use in high speed internal combustion engines, the steps which include pressing a mixture comprising a preponderating proportion of iron powder, about 1 to 10% of lead powder, and about 1.5% of graphite, to a specific weight of about 6.3 to 6.5, 55 sintering the mass at about 1,000 to 1200° C., subsequently again pressing the mass at a temperature of about 900 to 1,000° at a pressure of about 85,000 to 100,000 lbs./in.<sup>2</sup>, and quenching the pressed mass in a liquid from a temperature of about 800 to 850° C.
5. A sintered piston ring composed principally of iron and containing 1 to 10% of lead, at least part of the lead being in the form of an iron-lead-carbon alloy, the carbon content being of the order of about .5%.
6. A quenched, sintered piston ring composed principally of iron and containing 1 to 10% of lead and having a granular structure of the type of pearlite and sorbite, at least part of the lead being in the form of an iron-lead-carbon alloy, the carbon content being of the order of about .5%.
7. A sintered piston ring composed principally of iron

and containing about 0.48 to 0.52% of carbon, 3.45 to 3.55% of lead, 0.36 to 0.41% of tin and 0.45 to 0.52% of copper, the ring having an elastic limit of about 82,000 to 89,000 lbs./in.<sup>2</sup>, an ultimate strength of about 106,000 to 109,000 lbs./in.<sup>2</sup>, and an elongation of 1.5 to 2, at least part of the lead being in the form of an iron-lead-carbon alloy.

8. A substantially non-porous sintered piston ring composed principally of iron and containing 1 to 10% of lead which at least in part is in the form of an iron-lead-carbon alloy, with a small quantity of at least one member of the group consisting of tin, antimony, manganese, chromium, nickel, copper and silicon, said ring having a lamellar pearlitic structure and a specific gravity of 7.6 to 7.7.

9. A substantially non-porous sintered piston ring composed principally of iron and containing 1 to 10% of lead which at least in part is in the form of an iron-lead-carbon alloy, with a small quantity of at least one member of the group consisting of tin, antimony, manganese, chromium, nickel, copper and silicon, said ring having a granular structure of the type of pearlite and sorbite and a specific gravity of 7.6 to 7.7.

**References Cited** in the file of this patent

**UNITED STATES PATENTS**

1,793,757 Smith ----- Feb. 24, 1931

|    |           |                                       |
|----|-----------|---------------------------------------|
| 5  | 1,974,173 | Calkins ----- Sept. 18, 1934          |
|    | 2,192,792 | Kurtz ----- Mar. 5, 1940              |
|    | 2,214,104 | Hildabolt et al. ----- Sept. 10, 1940 |
|    | 2,275,420 | Clark et al. ----- Mar. 10, 1942      |
|    | 2,319,373 | Tormyn ----- May 18, 1943             |
|    | 2,327,805 | Koehring ----- Aug. 24, 1943          |
|    | 2,342,799 | Goetzel ----- Feb. 29, 1944           |
|    | 2,386,604 | Goetzel ----- Oct. 9, 1945            |
| 10 | 2,401,483 | Hensel ----- June 4, 1946             |
|    | 2,409,307 | Patch et al. ----- Oct. 15, 1946      |
|    | 2,411,073 | Whitney ----- Nov. 12, 1946           |
|    | 2,435,511 | Rice ----- Feb. 3, 1948               |
|    | 2,518,253 | Reis ----- Aug. 8, 1950               |

**FOREIGN PATENTS**

|    |         |                                   |
|----|---------|-----------------------------------|
| 15 | 609,689 | Great Britain ----- Oct. 5, 1948  |
|    | 625,397 | Great Britain ----- June 27, 1949 |

**OTHER REFERENCES**

|    |                                                                                                                     |  |
|----|---------------------------------------------------------------------------------------------------------------------|--|
| 20 | Metal Powder Report, I, 1947, pages 70 and 89.                                                                      |  |
|    | "Powder Metallurgy" by H. H. Hausner, page 128 (Table 41), published 1947 Chemical Publishing Co. (Brooklyn, N. Y.) |  |
| 25 | Goetzel: Treatise on Powder Metallurgy, Interscience Publishers, New York city, 1950, vol. 2, pages 522-523.        |  |